

W. D. COOLIDGE.

TUNGSTEN AND METHOD OF MAKING THE SAME FOR USE AS FILAMENTS OF INCANDESCENT  
ELECTRIC LAMPS AND FOR OTHER PURPOSES.

APPLICATION FILED JUNE 19, 1912.

1,082,933.

Patented Dec. 30, 1913.



Witnesses:

George H. Pilden  
J. Ellis Glen

Inventor:

William D. Coolidge,

by *Albert G. Davis*  
His Attorney.

# UNITED STATES PATENT OFFICE.

WILLIAM D. COOLIDGE, OF SCHENECTADY, NEW YORK, ASSIGNOR TO GENERAL ELECTRIC COMPANY, A CORPORATION OF NEW YORK.

## TUNGSTEN AND METHOD OF MAKING THE SAME FOR USE AS FILAMENTS OF INCANDESCENT ELECTRIC LAMPS AND FOR OTHER PURPOSES.

1,082,933.

Specification of Letters Patent. Patented Dec. 30, 1913.

Application filed June 19, 1912. Serial No. 704,580.

To all whom it may concern:

Be it known that I, WILLIAM D. COOLIDGE, a citizen of the United States, residing at Schenectady, county of Schenectady, State of New York, have invented certain new and useful Improvements in Tungsten and Methods of Making the Same for Use as Filaments of Incandescent Electric Lamps and for other Purposes, of which the following is a specification.

This application is in part a continuation of my prior applications, Serial Number 324,335, filed July 2, 1906; Serial Number 521,220, filed October 6, 1909; Serial Number 545,274, filed February 23, 1910; and Serial Number 577,353 filed August 15, 1910.

My invention comprises a new incandescent lamp filament of drawn wire made from the metal tungsten, and a process of producing the same. I have been able to produce from this refractory, brittle, non-ductile and generally unworkable metal a wire which is tough, fibrous and elastic and of high tensile strength, and have thus been able to facilitate the manufacture and improve the quality of tungsten incandescent electric lamps.

The wire produced by my invention has found various other applications, and may be used wherever high tensile strength, freedom from corrosion, or ability to withstand high temperatures are of value. So also the new material of which the wire consists, fully worked ductile tungsten, has in other mechanical forms a wide variety of useful applications. Further, an incidental but valuable new product is found at an intermediate stage of my process, in tungsten which is wrought, but in which the working process has been interrupted before the above described properties have fully developed but at a point where desirable properties not found in any tungsten of the prior art have been developed to an amount sufficient for the purposes for which the material in question is to be used.

The metal tungsten is described in standard works on chemistry and metallurgy as obtained in the form of a steel-gray to black powder, having a fusing point of about 3200 degrees C. It is stated to be entirely non-ductile. Thus, for example, Roscoe and Schorlemmer's *Treatise on Chemistry*, vol. 11, p. 1058, published in 1907, cites the

work of Moissan, but states that: "The purest forms of tungsten at present obtainable are hard and brittle, and are not ductile either at ordinary temperatures or when heated." De Lodyguine's Patent No. 575,002, referring to tungsten, states (page 1) that it is "almost absolutely non-ductile" and "cannot be drawn out into wires in the manner employed in operating on ductile metals". Also, the British patent of Siemens & Halske Aktiengesellschaft, No. 5387 of 1908, and British patent of Consortium fur Elektro-Chemische Industrie of Nurnberg, Germany, No. 3938, of 1907, state that tungsten is non-ductile and cannot be drawn into wires.

Up to the time of my present invention all efforts to work the metal have failed, and no one had succeeded in modifying its characteristic hard brittle structure. Incandescent lamp filaments had been made of tungsten by means of a sintering process, that is, by pressing up tungsten powder with or without a binder into the desired shape, and then consolidating it at a high temperature by passing electric current through it. Filaments so formed have been of exceedingly low strength and very brittle.

I have discovered a process by which tungsten bodies, when prepared under certain conditions, as will be hereinafter more fully described, can be mechanically worked as by hammering, swaging, rolling and drawing, and have further discovered that when this mechanical working is carried on while the metal is heated to temperatures within certain maximum and minimum limits and is continued long enough, such bodies will be converted from their original crystalline character to a condition having all the characteristics of a ductile metal. In other words, the repeated hot working so changes the metal that it acquires tensile strength and also becomes pliable and ductile at ordinary or room temperatures, and if the mechanical working is carried sufficiently far, and under proper conditions, the tensile strength of the metal may become equal to or greater than that of the best steel. I have thus not only devised a new process by which it has become possible to work tungsten, as by hammering it or rolling it into the desired form, and by drawing it into fine strong wire, but I have

also produced by the operation of this process a new product, viz: wrought tungsten, and, if the process be carried far enough, ductile tungsten, a material having properties and utilities different from those of any previously known substance. When it is desired to produce from this material an incandescent lamp filament, or any other body which in normal operation is to be operated at high temperatures, I use a special mode of preparation in order to minimize the tendency of the tungsten to revert to a brittle crystalline form. When this crystallization becomes excessive the crystals may, in the case of a filament, become so large as to extend across the entire section of the filament and thereupon the sections may move laterally upon each other and produce the condition known as "offsetting". I shall hereinafter describe more in detail the special method which I employ for minimizing the loss in ductility and for preventing this offsetting effect.

My process divides itself into two stages, first the preparation of an ingot or billet of tungsten, and second the working of the ingot, and I find that the more successfully the ingot is prepared the more quickly and readily it can be worked. Also, by using certain precautions in working I am able to handle ingots which have not been prepared in the best possible way. I have no doubt that with the progress of the art improvements will be made in my process whereby the ingot will be so prepared that its working becomes much easier than it now is, or whereby, through improvements in the working, less care and skill will be required in the preparation of the ingots. I will, however, first describe in detail a process which I have worked successfully on a large scale for the production of drawn tungsten wire of the highest quality suitable for filaments for incandescent lamps and by means of which a single tungsten wire seven miles long has been produced, and will thereafter describe certain of the numerous modifications of the process, within the scope of my invention, which may be resorted to as occasion requires.

In describing this process I will refer to the accompanying drawings in which—

Figure 1 shows a swaging machine, Figs. 2 and 3 are detailed views showing different forms of swaging dies; and Fig. 4 is a view of one form of wire-drawing apparatus, and Fig. 5 shows an electric furnace, and Fig. 6 is a view of an incandescent lamp made in accordance with my invention.

Starting with tungstic oxid ( $WO_3$ ) as pure as commercially obtainable, I dissolve it in ammonia water and thus form ammonium tungstate, which is purified by crystallization over a steam bath and is then,

after washing by distilled water and drying, decomposed by the application of moderate heat, say 400 to 500 degrees C. which drives off the ammonia and leaves purified tungstic oxid. The tungstic oxid thus purified is heated in a gas furnace for about five hours in a covered Hessian or Battersea crucible of the ordinary and well known type, after which step it is found to be coarser and of higher density and to contain matter, probably volatilized from the crucible, the effect of which, as will be hereinafter explained, is beneficial. The substances thus added to the oxid of tungsten, which for convenience I may designate as additions, consist largely of alumina, and silica. I have obtained best results when these additions occurred in the proportion of from 0.8 to 1.5 of one per cent.

If on analysis it is found that less than 85 0.8 of one per cent. of additions is present, the operation of firing in the Hessian or Battersea crucible is repeated as many times as may be necessary, a new crucible being used each time. The material, which 90 has somewhat melted and agglomerated into a mass, is ground after each firing.

The next operation is performed in a tube, for example of porcelain or fused quartz, having a diameter of one and one-half inches and a length of two feet. This tube is packed nearly full of tungstic oxid except that clear spaces are left at each end, and the tube is gradually raised by suitable gas burners or by electrical heating, 106 in six or seven hours, to a temperature which may be between 900 degrees C. and 1150 degrees C. I may if preferred use the type of furnace described by Winne and Dantszen in the *Transactions of the American Electrochemical Society*, vol. XX, 1911, pp. 289-90. Crystallinity in the metal powder is to be avoided and this result is aided by this slow raising of temperature. Pure, dry hydrogen passes through the tube during this heating operation for a period of say six to fifteen hours, and is preferably introduced through a small passage formed in the upper part of the charge next to the containing tube; which arrangement leaves 111 a thick body of the charge to be acted upon by the hydrogen. In this operation the tungstic oxid, or as it is called the "yellow oxid," is progressively reduced to the blue oxid and then to the brown oxid and then to the pure metal. The powdered tungsten thus formed is inserted, in weighed quantities, into a steel mold and is by means of a hydraulic press pressed into sticks or rods which may for example be  $\frac{1}{4}$  of an 112 inch square and six inches long, though good results have also been obtained with octagonal rods.

The mold is of extreme strength and rigidity and is arranged to apply the pres- 134

sure transversely of the stick to be formed. The powder is evenly placed in the mold so that the sticks shall be of uniform density from end to end.

5 When the pressure is removed the mold is split or opened and the pressed tungsten stick is gently slid on to a strip for example of molybdenum or tungsten and introduced into a tube of some such material as porcelain or alundum electrically heated by a winding of tungsten or platinum wire, in which apparatus the tungsten stick is fired in an atmosphere of hydrogen to a temperature of say 1200 degrees C., for from ten minutes to an hour, or long enough to permit the sticks to become strong, so that they may easily be handled. The molybdenum support may be withdrawn when the stick has been 20 brought to a bright red heat.

The pressing operation which I have just described is performed with dry tungsten powder but I may if desired use a binder which must afterward be removed. If the 25 binder is carbonaceous, the carbon may be removed by heating the sticks in moist hydrogen or if desired in hydrogen containing a small amount of air.

If the tube in which the heating or firing 30 operation is performed is made of porcelain, I fire the stick on a "boat" of suitable material such for example as molybdenum.

The fired sticks are then placed, one at a time, in a closed treating vessel, ordinarily 35 of copper and similar to those commonly used in sintering tungsten filaments, but larger and of more rugged construction, through which hydrogen or other reducing atmosphere is constantly passed, and an 40 electrical current is passed through them sufficiently intense to raise them to a blinding white heat. This sinters the stick and converts it into a coherent slug of metal. While in the treating vessel the sticks are 45 held in water-cooled spring clamps, one of which is carried by a fixed support while the lower one dips into a water cooled pool of mercury so as to adjust its position as the stick shortens up during sintering. In some 50 cases I water cool the bottle itself, and I find it best to cover the lower edges of the bottle with a mercury seal.

I prefer with the  $\frac{1}{4}$  inch rod six inches along to sinter at 1700 to 1800 amperes (alternating) for fifteen minutes, the current being gradually raised to this point in say about five minutes, and then to reduce the current by degrees until at the end of one minute or more it is cut off altogether, whereupon the rod may be withdrawn as soon as it cools sufficiently to allow the treating vessel to be opened. This slow reduction of the current is intended to prevent a sudden reduction of gas pressure in the 65 treating or sintering vessel, which would

tend to draw in air and produce an explosion. After the sintering operation, the ends of the slug held by the clamps and therefore but partially sintered, are broken off. This completes the preparation of the slug or 70 billet.

The next step is the mechanical working, which, in the particular process I am now describing, is carried on as follows: In Fig. 1 A is a swaging machine which may be of 75 the general type shown in United States patent to Dayton, No. 515,576, February 27, 1894. In this machine the head B is rotated and a pair of dies each like the dies shown for example in Fig. 2 or Fig. 3 are brought 80 together and then separated several times in each revolution. The head B carries the swaging dies and their operating mechanism and through the machine extends a horizontal passage D for receiving the work as it 85 passes through the dies. The dies C, unlike the ordinary swaging dies, have very short faces E, about equal in length to the diameter of the tungsten piece passing between them. The edges C' in the working surfaces 90 are rounded or "backed off" to keep the die from digging into the rod. In some cases a die may be used having a peculiar form of face, shown in Fig. 3, in which the edges of the striking portion or face of the die are 95 rounded off gradually.

In Fig. 5, F is a tube furnace of the type described in the Winne and Dantszen article above referred to. It consists of a tube G of alundum or porcelain; a winding of wire 100 H of platinum or preferably tungsten or molybdenum through which an electric current may be passed, and a heat insulating cover K of magnesite, fine silica or other suitable material held by a suitable shell or casing of asbestos, fire brick, sheet iron or the like. Hydrogen is passed through the tube G in any suitable way as by the pipe I. The operator grasps with a pair of tongs one of the tungsten billets or slugs and inserts 105 it in the furnace, which is in some convenient location near the swager, and leaves it there until it attains a high temperature, say 1300 to 1700 degrees C., and at which, when the billet is removed from the furnace into the 110 open air, it gives off a cloud of volatilized 115 oxid of tungsten. He then takes the smoking hot billet with the tongs and quickly thrusts it as far as he can into the swaging machine and as quickly withdraws it. The 120 swaging machine runs at high speed and care should be taken to keep the slug in rapid motion into and out of the dies so as not to cool it materially. The dies are chosen so that each shall produce only a slight decrease in the cross-section of the billet and if the billet is square it is necessary to use care in passing from the square to the circular form, which form is of course produced by 125 the action of the dies, and ordinarily the 130

dies should be so adjusted that several passes through different dies occur in the production of the circular form.

The billet after being inserted in the first 5 dies is reheated in the furnace, then grasped by the other end and, without changing the dies, quickly thrust into the swaging machine, and quickly withdrawn as before. As many 10 billets as may be ready for treatment are thus manipulated and then the dies are removed and other dies are inserted arranged to produce a somewhat smaller section, and so on.

Starting with the  $\frac{1}{4}$  inch square billet, I 15 am able with five (5) passes through the machine to obtain a circular rod of 210 mils. in diameter. From 210 mils. to 60 mils. I ordinarily proceed by ten steps. As the billet 20 becomes longer and smaller in diameter I may use a gas furnace or heater instead of the electric furnace and a smaller size swaging machine, and the billet, which is now a wire or rod, is drawn by the action of mechanically driven feed rollers through the 25 gas flame of a gas furnace, which is then located in front of the swager, and through the swaging dies, passing completely through the opening corresponding to D in Fig. 1, and when this arrangement is adopted only 30 one pass is necessary with each die setting.

The swaging operation is continued, with continual reduction of the dies, until in six 35 or seven more operations the wire has been reduced to thirty mils. diameter. The temperature to which the rod is heated, which was originally at white heat, is reduced at the diameter of about 40 mils. to a yellow red and this temperature is maintained to the end of the swaging operation; that is to 40 say until a diameter of 30 mils. has been reached. At or by this time the material has become ductile at room temperature and can be bent and otherwise manipulated.

The wire drawing die L, Fig. 4, consists 45 of a drilled diamond set in metal, held by supports M and heated by a number of gas jets N. The wire is pointed by dipping the end in fused potassium nitrite, as is disclosed in the Whitney Patent No. 1,008,762, 50 and the pointed end is then inserted in the die and grasped by the clamp O, which may be heated at the point where it holds the wire by a gas jet P, or the operator may merely grasp by a pair of pliers the end of 55 the wire where it emerges from the die and pull a few feet of it through the die and attach the end to a spool or spindle which is revolved by power. In this manner the whole length of the wire resulting from the 60 swaged billet is drawn through the die, but before it passes through the die it should pass through a bath of a material known as aqua dag, which I understand is a deflocculated graphite suspended in water, or of

oil dag, which is a similar preparation in which oil is used instead of water as a suspending medium. This is done in the manner set forth in the Dempster Patent No. 1,022,182. The die should be at a temperature of 600 to 650 degrees C. and the wire 70 should be red hot both when going into the die and when emerging therefrom.

Further reduction is accomplished in the same way, the dies varying by one mil. steps down to 14 mils., making 16 drawing operations from 30 to 14 mils. At 14 mils. or thereabout the temperature of the dies may be reduced below a red heat, but the wire itself is run red hot through the die down to sizes approximating 3 mils.

From 14 to 5.5 mils. the dies should vary in steps of one-half of a mil., making 17 additional operations; from 5.5 mils. to 4 mils. there are five operations with steps of  $\frac{1}{2}$  of a mil.; from four mils. to 2 mils. there are 8. 0.2 of a mil. drafts; and from 2 mils. to 1.4 mils. there are six operations with steps of  $\frac{1}{16}$  of a mil.; and from 1.4 mils. to 0.5 mil. there are 18 operations with one twentieth of a mil. draft.

As the wire reaches smaller sizes the method of pointing described in the Whitney patent above mentioned becomes inconvenient, and instead the wire is dipped in a strong solution of potassium cyanide, and current is passed through the wire in such a direction as to make it an anode. Of course the wire drawing may be stopped at any stage according to the size of wire desired.

The metal obtainable as the ultimate result of the operations above described is a new product differing radically from any form of tungsten heretofore obtained. Not only is it pliable and ductile at room temperature, but it is strong and tough. It is substantially non-oxidizing in moist air at ordinary temperatures and resists the action of acids to an unusual degree. Its specific gravity is higher than that of sintered tungsten and has been found in certain samples 1 to run from 19.15 to 19.3. It has an exceedingly high tensile strength, as high in particular samples of .001" diameter as 600,000 to 650,000 lbs. per square inch, is non-magnetic and not easily corroded, and is elastic 1 and resilient.

The material has a wide variety of technical uses. If used for filaments of incandescent lamps, it may be mounted as described in the Feuerlein Patent, No. 819,009, April 25, 1906, as shown in Fig. 6 of the drawings hereto attached. Before this is done, however, the wire may if desired be freed from impurities on its surface in some suitable manner as by passing it through a bath of hot caustic soda and then through a suitable wiper. When run in the lamp the drawn tungsten filament made as described

loses much of its strength but is then, if carefully prepared in accordance with the directions herein given, nevertheless a much stronger filament than that made by ordinary squirting processes. To guard against this loss in strength, the filament should not be run at a very high temperature in the lamp until the lamp has been sealed off from the evacuating pump.

10 If my new material is used as the target of an X-ray tube it gives the tube a life and constancy of vacuum far superior to that possible by the use of a target of any other known material. It presents many advantages for use as contacts for magnetos and other devices where making and breaking of a circuit occurs, and is for such purposes far preferable to platinum and other materials now in use.

20 For certain applications the complete working process resulting in an entirely ductile metal of great tensile strength is not required. For example, after a certain amount of rolling or swaging, depending on 25 the amount of softness and strength which the metal should have for the purpose for which it is to be used, or without any swaging or rolling whatever if great strength is not necessary in the finished product, I can 30 heat the metal, for example in an alundum tube furnace, and hammer it into any desired shape, shear it, or roll it into plates, and from these plates I can punch parts of 35 any desired configuration provided that the material has been prepared in accordance with the directions above given, and that the operation, whatever it may be, is performed, except in cases where the fiber has been very 40 thoroughly developed by long-repeated mechanical working, at a sufficiently high temperature. When I have desired to produce a number of identical pieces I have resorted to a drop-forging operation.

The metal produced even by incomplete 45 working differs markedly from any form of tungsten heretofore known, for example, it is stronger and tougher and less liable to cracking on unequal heating and cooling. When the working is fairly complete, the 50 crystals characteristic of sintered tungsten have been deformed, broken up and elongated to such an extent that the structure is fibrous. When the working is less complete the crystals are broken up, though to a less 55 extent, and are deformed as by elongation or flattening, according to the nature of the working process. When, for example, the billet is hammered into a plate or sheet, the crystals are found to have become flattened.

60 An important point in practising the above described method of carrying out my invention is the temperature to which the metal is raised and at which the several operations are carried on. Where it is desired

that the resulting metal shall have the properties of a wrought metal more or less pliable and ductile at ordinary temperatures, it is not only necessary to repeat the mechanical working a large number of times, but it is necessary to keep at all times with- 65 in a certain range of temperature at least during the later stages of working. It is necessary, on the one hand, that the temperature be high enough to make it possible to mechanically work the body, but, on the other hand, too high a temperature is objectionable because if the temperature is too high a tendency appears to lose fiber already acquired and to pass to a state of brittleness from a state of ductility. The range 70 of temperatures within which properly prepared tungsten bodies may be worked to produce ductility at room temperature in accordance with my invention varies with the particular material used, but according to 75 my experience heating the metal to or working it at a temperature corresponding to white heat and materially in excess of about 1500° C. will tend to prevent, with any tungsten metal which I have been able to produce, the formation of fiber and will tend 80 to destroy fiber which has been produced by previous working. On the other hand, an excessive amount of mechanical working tends to cause the bodies to become so 85 fibrous and hard as to split up and break. I have found that this result may be obviated by carrying on the mechanical working during the early stages at such temperatures as 90 enable the body to be worked and reduced in size but without causing any special change in the structure of the metal. These 95 temperatures may correspond to a white heat or thereabout but should be above a temperature which I estimate at about 1500 100 degrees C. At the proper stages of the process the temperature is reduced to 1200 degrees C., or lower, whereupon as the mechanical working progresses the improvement 105 in the structure of the metal begins. 110

The preparation of a tungsten body which is to be mechanically worked is an important feature of my invention, for it is not every tungsten body which is susceptible of mechanical working. For example, Moissan states (*Comptes Rendus*, vol. 123, pp. 115 13-16, 1896-7) that he obtained by heating tungstic acid and sugar carbon in a carbon crucible an ingot or melt which presented well fused superficial portions, but which 120 was porous in its interior portions. Of this product Moissan says that when it is in a porous condition it has, like iron, the property that it may be consolidated (*la propriété de se soudre à lui-même*), by hammering much below its point of fusion. 125

Subsequent investigators have expressed the opinion that the material which Moissan

- obtained was not pure tungsten, but tungsten contaminated by carbon. Certainly there is no indication that by hammering Moissan was able to do anything more than to close more or less the pores of the porous material, whatever it may have been, to which he refers; nor is there any indication that when he had gone thus far he had produced a material which could be worked.
- 10 I have found that in order that the swaging process may be carried on successfully it is necessary that the tungsten should be in a certain physical or molecular condition, such as is brought about by the treatments 15 which I have discussed above. I find it particularly advantageous to work with tungsten powder which is coarse as distinguished from the exceedingly fine and impalpable powder such as has been used in 20 the manufacture of lamp filaments. The operation of heating in the Battersea crucible coarsens the powder, as does also the reduction operation, particularly if it be carried on in the manner described, and if the 25 hydrogen be passed rather slowly through the reduction furnace. While my invention has made it possible with certain precautions to work fine grained metal (especially if it contains oxids, which delay sintering), 30 as by excessively small drafts and by surrounding the rod with a sheath or casing of some other metal, the condition of the tungsten which is characteristic of the coarse powder is one which is peculiarly adapted 35 to the successful practice of my invention.
- Though the operativeness of my invention obviously does not depend upon any theory of operation, I may state that I am at present of the opinion that the difficulty 40 which is observed in swaging the rods pressed from the fine powder may well be due to the presence in such rods of certain impurities, probably gaseous impurities, as for example oxygen, which would probably 45 occur as an oxid of tungsten. The atomic weight of tungsten is so high (184) that even a small percentage of oxygen will cause a very large percentage of the tungsten to exist as the oxid. It seems probable that in 50 the sintering process the gaseous impurities are expelled more readily from the rod pressed from coarse powder, while in the case of a rod pressed from fine powder the tendency is to sinter quickly on the outside 55 and so prevent or greatly retard the escape of impurities. This hypothesis is consistent with the fact that the smaller the rod the less the importance of using a specially prepared material.
- 60 My opinion that the coarseness of the structure has some effect on the sintering operation is confirmed by the fact that the effects characteristic of coarse grained powder are produced by any process by which a 65 rod is formed which is coarse at the time it

is exposed to the sintering operation. For example, I have produced rods from exceedingly fine tungsten powder which, after sintering, swage very well, by carrying on the baking operation in an iron tube furnace. The rods are packed in the tube in powdered silica and hydrogen is passed through the tube. The tube is heated by gas flames for 8 or 10 hours to a rather low temperature. This baking operation produces a rod of coarse grained structure, probably because of the fact that the oxid, naturally existing in considerable quantities in so fine a powder, requires prolonged heating to effect complete reduction and coarsens during this prolonged heating in the oxid stage.

70 It is desirable in all cases that the sintering operation should take place slowly, in order to give time for the action of the 75 hydrogen to penetrate through the entire mass, and to facilitate the escape of impurities, as well as to prevent the center of the 80 rod, by a too rapid increase of the heating current, from becoming much hotter than the outside and actually melting and running out.

85 The ultimate temperature reached in the sintering operation should be very high, a dazzling white heat probably not far from 90 2800° C. It is difficult to give any general rule, except to state that if an insufficiently high temperature is reached the rod will break up in the swaging machine. Such a 95 rod ordinarily shows a very finely grained fracture, while my experience is that the rods which are capable of being worked easily show a somewhat coarser and more 100 crystalline fracture.

105 It is my belief that certain impurities in the sintered rod, such for example as oxygen and carbon, are highly detrimental and prevent the swaging operation from being successfully carried on. On the other hand I have stated above that certain additions are 110 absorbed from the Hessian or Battersea crucible operation, and I find that these additions do not prevent the swaging while they exercise a highly beneficial action where the tungsten is to be exposed for long periods of time to high temperatures, particularly in the form of incandescent lamp filaments. It may be that "offsetting," a phenomenon which as above explained is characteristic of some drawn wire lamp filaments, is due to the crystallization of the metal and the segregation of impurities, whereby spots are developed at which this side slipping or offsetting occurs, and that the presence of the additions introduced 115 from the Hessian or Battersea crucible retards or interferes with the diffusion of such impurities and thus retards crystallization. It is a fact that this treatment prevents off-setting.

I have succeeded in preventing offsetting in drawn tungsten filaments without using the Battersea crucible process by mixing with the tungsten powder certain refractory materials such as the oxides of thorium, zirconium, yttrium, erbium, didymium, or ytterbium. I have used with especial success thorium nitrate, which gives thoria when decomposed. A small amount of the above mentioned oxides, or of compounds or solutions which upon heating or other treatment will yield these oxides, may be mixed with the tungstic oxide before reduction or with the metal powder after reduction; or may even be introduced after the metal has been made into a stick, either by soaking the stick in a solution of a suitable substance or by heating the stick in the presence of a suitable material in the vaporous condition.

When thorium nitrate is used, for example, I employ an amount which is equivalent to 2% or less of thoria referred to tungsten. The essential point seems to be that the material should be introduced before the tungsten is sintered. Such additions, particularly in the case of a filamentary body, may actually produce a certain amount of ductility and flexibility in the sintered filament without mechanical working. Usually, however, instead of directly adding these substances, I prefer to employ the treatment above described of simply firing the tungstic oxide in a Hessian or Battersea crucible, for this treatment is simple, successful and reliable.

While I have referred to a considerable extent to the manufacture of ductile tungsten in which so-called additions are introduced at some stage of the process in order that the resulting product may be especially valuable when used for filaments of incandescent lamps, and in connection with other uses where the metal is to be exposed for long periods of time to high temperatures, nevertheless operative and useful incandescent-lamp filaments may be made by carrying out my process as herein described, omitting the additions whether produced by direct introduction of additional material, as above described, or by the Battersea-crucible process; and where it is sought to obtain ductile tungsten for uses in which it is not likely to be exposed to high temperatures, the introduction of such additional substances may be entirely unnecessary. I do not however wish it to be understood that metal prepared with the additions can only be used in incandescent lamps and for similar purposes, as such metal can, as far as my present knowledge extends, be used for any purpose to which the ductile tungsten prepared without the use of the additions is applicable.

In connection with the swaging operation it should be noted that I have departed radi-

cally from the ordinary swaging process, in which the dies are long and the metal is held a considerable time in the machine or passed very slowly through it, so that a number of blows are struck at the same place on the metal, and a smooth surface is produced. I find it highly desirable, particularly in the earlier stages of the swaging process, to use a die with a very short working face such as I have shown in the drawings, and to pass the metal through the machine at high speed and so that it is still highly heated when it emerges from the dies. Indeed, it is best not to allow two successive blows to be struck at too closely overlapping places, because each impact of the die abstracts a certain amount of heat from the material and unless this precaution be observed there is great danger that a blow will be struck upon metal which is too cold to endure it without cracking. Preferably, then, the metal emerges from the swaging machine, not smooth, but showing every distinct blow of the hammer, and therefore with an irregular wavy surface.

The swaging operation, though the most successful at the moment, is not the only operation by which my invention can be practised. For example, I have succeeded, without any swaging operation whatever and using only wire-drawing dies, in producing perfectly ductile tungsten. In this case I have begun the operation with sintered conductors of relatively small size. For example, I have used ordinary sintered series tungsten incandescent lamp filaments of the diameter of 25 mils. Where the original body is so small in diameter it is relatively easy to expel injurious impurities in the sintering process, and the devices above described to facilitate this end, which are of importance in the case of the larger bodies which are required for economical large-scale production of lamp filaments, or for the preparation of larger articles, such as X-ray tube targets, projectiles, contacts, etc., become relatively unimportant where the original sintered body is of sufficiently small diameter. I point these filaments by the process of the Whitney Patent, No. 1,008,762, above referred to, and carefully insert the point into a die which is heated to 600 to 650° C. The pointed end is then seized with hot pliers (otherwise it would break) and the filament is then with great care and with a regular steady pull drawn through the die, the diameter of which should be not less than  $\frac{1}{2}$  a mil (.0005 inch less than the maximum diameter of the filament at any point. The filament is then in a similar way drawn through a die having a diameter of  $\frac{1}{2}$  a mil (.0005 inch) less than that of the first die, and so on down to 13 mils. Below this size the dies should vary in steps of one-quarter of a mil until a size of say four mils. is

reached when the dies should then vary by one-eighth of a mil. or less. As the wire becomes smaller the temperature of drawing is reduced; at 18 mils. or thereabout the temperature is reduced from 600 or 650° to 500° C.; at 10 mils. the temperature is reduced to 400° C. The dies are lubricated with aqua dag or oil dag, as in the wire-drawing process first described. After such a 25 mil. filament has been drawn to a diameter of 7 mils., it can, at room temperature, be bent around the finger without breaking, and will readily take a permanent set. As the tungsten is still further worked by drawing down to smaller sizes, the fibrous condition becomes more and more developed and the wire becomes more and more pliable, until, at a diameter of about 4 mils., it is in every sense ductile material, and could if desired be manipulated as any other ductile metal, and drawn through dies not heated above room temperature, though I ordinarily heat the dies during the last stages of the drawing process as well as during the first stages, since by the application of heat the drawing is rendered somewhat easier.

As a convenient means for keeping the tungsten hot during the drawing operation, I may, if desired, pass current through the material under treatment. The die and the portion of the wire which is hot may be enclosed in an evacuated space or in a hydrogen or other reducing atmosphere, although I do not find it necessary to do so. The lubricants mentioned herein themselves materially assist in protecting the wire from oxidation. So also I have succeeded in producing ductile tungsten by a rolling process. In carrying out such a process, at least until the metal has acquired a considerable amount of fiber, the rolling operation should be carried on with the metal at a high temperature, preferably between what is known as "bright red heat" and "white heat," and that the metal should retain this temperature as long as the rolls are acting upon it. Excessive temperatures, such as temperatures above 1500° C., are objectionable for the reasons and to the extent already explained. The rolls naturally abstract heat rapidly and therefore the metal should pass through the rolls at very high speed; it is also essential that the draft of the rolls should not be too great. Also, at least during the later stages of rolling, the temperature should not be higher than about 1200° C.; and preferably in the neighborhood of 1000° C. When a sufficiently fibrous condition has been obtained by rolling, the metal may be run through dies as above described, or the working may be continued exclusively by rolling.

What I claim as new and desire to secure by Letters Patent of the United States, is,—

65 1. The process of producing tungsten hav-

ing a fibrous structure which consists in repeatedly hot working a crystalline body of tungsten until the crystalline structure is broken down and a fibrous structure developed.

2. The process which consists in agglomerating tungsten powder, sintering the body thus formed, subjecting it to repeated hot working, and continuing such hot working until the body remains ductile when cold.

3. The process of producing ductile tungsten wire which consists in forming a sintered body of tungsten, hot swaging said body repeatedly until it becomes fibrous in structure, and then further reducing it by hot drawing.

4. The process of producing ductile tungsten wire, which consists in first forming a sintered body of tungsten free from oxygen carbon and other impurities which would render the body unworkable mechanically, then hot swaging such sintered and purified body repeatedly until it becomes fibrous in structure and then further reducing it by hot drawing.

5. The process which consists in mechanically working while hot tungsten which is brittle at room temperature until it becomes pliable at room temperature.

6. The process of forming bodies of coherent homogeneous tungsten which consists in agglomerating tungsten powder, sintering the body thus formed, and then subjecting it to hot mechanical working to such an extent as to improve the internal structure and to bring the body into a shape adapted for use in the arts.

7. The method which consists in first producing a body of tungsten sintered or compacted throughout and free from such impurities as would render the body unworkable mechanically, and then hot working said body to such an extent as to deform its crystalline structure and to bring it into a shape adapted for use in the arts.

8. The method of producing pliable tungsten wire for lamp filaments, which consists in first producing a body of tungsten in a sintered state and free from oxygen carbon and other impurities which would render the body unworkable mechanically and then subjecting this sintered and purified body to mechanical working many times repeated, with gradual reduction in diameter and elongation in length.

9. The method which consists in agglomerating relatively coarse tungsten powder into a porous mass, eliminating harmful impurities and compacting the mass by a sintering operation, and then mechanically working the resulting body while hot into the desired shape.

10. The method of producing ductile tungsten which consists in sintering an agglomerated mass of tungsten particles or

- powder into a dense coherent and homogeneous form in such manner as to allow elimination of harmful impurities, and then mechanically working said body until it is brought into the desired condition. 5
11. The process which consists in agglomerating tungsten powder, treating the body thus formed so as to eliminate any oxygen present therein and to produce therefrom a 10 sintered body, and then hot working such sintered body.
12. The process which consists in reducing tungsten oxid to coarse tungsten powder, agglomerating said powder into a coherent porous body, heating said body to drive out impurities and sinter the body, and then subjecting the body to hot mechanical working. 15
13. The process which consists in firing tungsten oxid in a refractory crucible of the Hessian or Battersea type, reducing the oxid to coarse metallic powder, agglomerating the powder into a coherent body, sintering the body, and then subjecting it to 20 hot mechanical working.
14. The process which consists in forming a body of tungsten powder containing additional material which will prevent coarse crystallization of the tungsten at high temperature, sintering the body, and then subjecting it to hot mechanical working. 25
15. The step in the preparation of tungsten bodies which consists in firing tungsten oxid in a refractory crucible of the Hessian or Battersea type, and subsequently 30 reducing the oxid to metallic tungsten powder.
16. The process which consists in producing tungsten containing beneficial additions, forming it into a billet, sintering it at high 35 temperature, and mechanically working it a great number of times at high temperature, and reducing the temperature during the working. 40
- 45 17. The method of producing bodies of tungsten pliable and ductile at ordinary or room temperatures from bodies of tungsten which are brittle at ordinary or room temperatures; which consists in heating said 50 brittle bodies to a temperature sufficient to render them susceptible of mechanical working, repeatedly working the bodies while so heated, and during at least the last stages of mechanical working carrying on the 55 working at temperatures such that the mechanical working has the effect of producing ductility in the finished product.
18. The method of producing bodies of ductile tungsten from bodies of tungsten 60 which are non-ductile, which consists in mechanically working the non-ductile bodies of tungsten within a temperature range at the lower limit of which the body to be worked is soft enough to be susceptible of 65 such working while the upper limit, at least during the later stages of the working, is sufficiently low to cause the body thus worked to retain to a greater or less degree the effect of the mechanical working.
19. The method of producing ductile tungsten which consists in repeatedly hot working a tungsten body within a range of temperature in which the body is sufficiently soft to be susceptible of such working, but maintaining the temperatures below those at 75 which the effect of the mechanical working is lost. 70
20. The method of producing a body of ductile tungsten from a body of tungsten which is brittle when cold, which consists in mechanically working said body while heated to a temperature at which the body is softened and finishing the mechanical working at temperatures below those at 80 which no ductility is imparted to the metal by the mechanical working. 85
21. The method which consists in mechanically working at a temperature above approximately 1500 degrees C. a tungsten body which is brittle cold, interrupting the 90 operation before the body is brought into the form ultimately desired, and completing the mechanical working at a temperature below 1500 degrees C.
22. The method of securing a ductile 95 metal body without previous melting of the metal, which consists in producing a compact body of metal from divided metalliferous material, consolidating said body by heating to a temperature less than the melting temperature and such as to produce a body of metal non-ductile when cold, subjecting the body to repeated mechanical working while in a heated condition, and continuing the working until the body is 100 ductile without the application of heat. 105
23. The method of securing a ductile metal body without previous melting of the metal, which consists in producing from divided metalliferous material a compact 110 body of metal, sintering said body and thereby producing a crystalline body brittle at room temperatures, and then subjecting the body to repeated mechanical working while hot, and continuing the working until 115 the metal remains ductile when cooled.
24. A wire formed of ductile tungsten.
25. An incandescent electric lamp having a filament of drawn tungsten wire.
26. Substantially pure tungsten having 120 ductility and high tensile strength.
27. A ductile tungsten wire having a fibrous structure.
28. A form of tungsten metal pliable at room temperature. 125
29. An incandescent electric lamp having a filament formed of ductile tungsten.
30. A lamp filament of tungsten which

resists offsetting and has high tensile strength.

31. A filamentary conductor of drawn tungsten so constituted as to be free from offsetting when operated as a filament of an incandescent lamp.

32. A filament for electric incandescent lamps consisting of tungsten wire which is pliable at ordinary or room temperature.

10 33. The material wrought tungsten, having a specific gravity of approximately 19

or greater, and capable of being forged and worked.

34. Wrought tungsten, a solid coherent material characterized by the presence of 15 crystals deformed by mechanical working.

In witness whereof, I have hereunto set my hand this 18th day of June, 1912.

WILLIAM D. COOLIDGE.

Witnesses:

NEWTON A. BURGESS,  
HELEN ORFORD.

#### DISCLAIMER.

1,082,933.—*William D. Coolidge, Schenectady, N. Y. TUNGSTEN AND METHODS OF MAKING THE SAME FOR USE AS FILAMENTS OF INCANDESCENT ELECTRIC LAMPS AND FOR OTHER PURPOSES.* Patent dated December 30, 1913. Disclaimer filed January 25, 1929, by the assignee, *General Electric Company*.

Hereby disclaims the subject matter of claims 14, 16, 24, 25, 26, 28, 29, 30, 31, 32, and 33.

Your petitioner further hereby disclaims the subject matter of claim 27, which reads as follows:

“A ductile tungsten wire having a fibrous structure.” except when the product defined in said claim 27 has been produced by the process disclosed in the specification of said patent, as more particularly defined in claim 5 of the said patent.

[*Official Gazette February 5, 1929.*]